

April 26, 1960

D. J. SCHMATZ ET AL

2,934,463

HIGH STRENGTH STEEL

Filed April 17, 1959

4 Sheets-Sheet 1



FIG. 1

D. J. SCHMATZ  
J. C. SHYNE  
V. F. ZACKAY  
INVENTORS

E. C. McRae  
BY J. R. Daubkner  
G. H. Oster  
H. L. Zerschling  
ATTORNEYS

April 26, 1960

D. J. SCHMATZ ET AL

2,934,463

HIGH STRENGTH STEEL

Filed April 17, 1959

4 Sheets-Sheet 2



FIG. 2

D. J. SCHMATZ  
J. C. SHYNE  
V. F. ZACKAY  
INVENTOR.

BY *J. C. Shyne*  
*D. B. Oster*

ATTORNEYS

April 26, 1960

D. J. SCHMATZ ET AL

2,934,463

HIGH STRENGTH STEEL

Filed April 17, 1959

4 Sheets-Sheet 3



FIG. 3

D. J. SCHMATZ

J. C. SHYNE

V. F. ZACKAY

INVENTOR.

BY *J. B. Faulkner*  
*J. H. Oster*

ATTORNEYS

April 26, 1960

D. J. SCHMATZ ET AL  
HIGH STRENGTH STEEL

2,934,463

Filed April 17, 1959

4 Sheets-Sheet 4



FIG. 4

D. J. SCHMATZ  
J. C. SHYNE  
V. F. ZACKAY

INVENTOR.

BY *J. B. Faulkner*  
*T. H. Oster*

ATTORNEYS

1

2,934,463

## HIGH STRENGTH STEEL

Duane J. Schmatz, Dearborn, John C. Shyne, Belleville, and Victor F. Zackay, Dearborn, Mich., assignors to Ford Motor Company, Dearborn, Mich., a corporation of Delaware

Application April 17, 1959, Serial No. 807,231

22 Claims. (Cl. 148—31)

This is a continuation-in-part of our application Serial Number 726,485, filed April 4, 1958.

This invention is directed to a class of high strength steels and to the heat treatment employed to obtain the optimum physical properties from these steels. This invention makes possible the production of very high strength steels in articles having a substantial minimum dimension as contrasted to wire and strip. The steels produced by this invention are characterized by a very high tensile strength and a high ratio of yield point to tensile strength. This invention is further concerned with a heat treating method in which the above enumerated valuable properties are obtained in combination with substantial ductility as expressed in terms of elongation and reduction of area so that products produced from such steel find ready commercial acceptance.

This invention is designed as an improvement upon the process described by Lips et al. in Metal Progress, August 1954, pages 103 and 104. This invention is also to be distinguished from the teachings of United States Letters Patent 2,435,511, issued February 3, 1945, to R. E. Rice and 2,717,846, issued September 13, 1955, to Harvey.

This invention has been developed for use with steels which exhibit a temperature region below the pearlite transformation temperature and above the bainite transformation temperature in which the metastable austenite is comparatively stable, even under conditions of substantial working for a protracted period of time. The following three steels are given by way of examples of steels possessing such a stable austenite.

|                 |       |      |       |
|-----------------|-------|------|-------|
| Carbon.....     | 0.49  | 0.60 | 0.33  |
| Manganese.....  | 0.41  | 0.39 | 0.23  |
| Phosphorus..... | 0.017 |      | 0.013 |
| Silicon.....    | 0.33  | 0.26 | 0.06  |
| Nickel.....     | 2.97  | 3.29 | 3.73  |
| Chromium.....   | 1.87  | 2.22 | 1.79  |

Chromium appears to be the most effective, most economical and generally desirable element whose addition to a steel composition will increase the temperature range covered by the temperature region mentioned supra and also increase the depth of such a temperature region along the time axis in the usual TTT diagram. These steels and their equilibrium isothermal transformation properties are detailed in a Supplement to Atlas of Isothermal Transformation Diagrams published in 1953 by the United States Steel Corporation at pages 216, 221 and 224 respectively. An inspection of the isothermal transformation diagrams presented for these steels will show that each steel is characterized by a temperature region adjacent 900° Fahrenheit in which metastable austenite can exist without transformation for at least an hour and in many cases for much longer periods of time under normal conditions. The behavior of these metastable austenitic steels under conditions of stress has been expounded upon at length by Bhattacharyya and Kehl in two scholarly articles published recently in the Transactions of the American Society for Metals. The first article appears in

2

the 1955 volume and begins at page 351 and the second article appears in 1956 and begins at page 234. These articles reflect the universally held opinion that the wealth of information presented in the conventional TTT diagrams while valid for normal conditions is completely inapplicable to metastable austenite while under working conditions. The data appearing upon pages 358 and 359 of the 1955 article is thought to be particularly enlightening. Here specifically dealing with an AISI 4340 steel a stress of only 60,000 pounds per square inch is stated to foreshorten the beginning of an isothermal transformation at 845° F. by a factor of four and to similarly effect the termination of the transformation time by a factor of ten thousand to one hundred thousand. Data of this type has discouraged the art from attempting extensive working of steels in the metastable austenitic condition since the stresses introduced by heavy reductions would far exceed the value of 60,000 pounds per square inch and the unwanted transformation of austenite into high temperature decomposition products seemed inevitable.

Despite this data, steel compositions exhibiting a wide bay between the pearlite transformation zone and the bainite transformation zone have been very heavily worked in this selected temperature region while in a metastable austenitic state and have remained austenitic for sufficient time to permit all necessary working operations, even including a reheating operation. The amount of plastic deformation has even been carried beyond the extreme value of ninety-three per cent with a rapid improvement being noted beyond twenty-five per cent reduction. After this extensive working the material is quenched to the martensitic transformation zone and permitted to transform to martensite. When properly tempered, the steel composition so produced demonstrates unique physical and microstructural characteristics.

To aid in an understanding of this invention four figures of drawing have been presented in which:

Figure 1 is an electron microscope photomicrograph of a typical steel composition produced according to the instant invention and magnified 40,000 times.

Figure 2 is a typical TTT diagram for a steel having a bay or deformation range in which austenite is metastable and can be heavily worked without inducing transformation in this temperature range to non-austenitic isothermal decomposition products. Particular attention is invited to the fact that the time scale along the abscissa is logarithmic. This is, of course, a normal showing and not to be applied to dynamic or working conditions. For the sake of clarity, a curve has been applied to this figure of drawing depicting a typical operation of the invention.

Figure 3 has been added to graphically depict the remarkable physical properties obtained upon tempering steel articles which have been drastically deformed in the metastable austenitic state and then quenched to give a predominantly martensitic structure. Attention is invited to the sharp increase in yield point of these steels as the tempering is increased. A steel of relatively low alloy content demonstrates a yield point of almost 400,000 pounds per square inch, while retaining an elongation of almost five per cent.

Figure 4 of the drawings is almost self-explanatory and has been presented to graphically illustrate the unexpected rise in both the tensile strength and yield point of tempered samples which have been very drastically worked in the metastable austenitic state.

Metallographically, the compositions produced by this invention may be described as an ultra fine grained martensite. The grain size of the martensitic structure which characterizes this invention is reduced by the mechanical deformation to an extent that the grain size in the finished article is less than one-half of the size which would be

obtained by the same treatment without the mechanical deformation. A typical individual martensite needle obtained by this invention exhibits a length of about three microns and a thickness of one-half micron. Without the mechanical deformation these dimensions would be numerically twice as great.

The following compositions were specifically investigated in the perfection of this invention:

| Code | Percent Carbon | Percent Nickel | Percent Chromium | Percent Silicon |
|------|----------------|----------------|------------------|-----------------|
| 179  | 0.98           | 3.96           | -----            | -----           |
| 802  | 0.28           | 4.63           | 1.42             | -----           |
| 803  | 0.32           | 4.55           | 1.42             | -----           |
| 842  | 0.35           | 4.60           | 1.46             | 1.78            |
| B10. | 0.37           | 4.80           | 1.45             | 1.68            |
| B11. | 0.38           | 4.78           | 1.48             | 1.59            |
| B12. | 0.40           | 4.75           | 1.45             | 1.55            |
| A25. | 0.44           | 4.49           | 1.41             | 1.40            |
| A26. | 0.49           | 4.50           | 1.44             | 1.43            |
| A27. | 0.52           | 4.53           | 1.42             | 1.47            |
| A28. | 0.57           | 4.67           | 1.38             | 1.48            |

In carrying out this invention a suitable steel composition is first austenitized by heating to a suitable temperature and then quickly brought into the selected temperature region by quenching in a liquid maintained at the proper temperature which should fall within the selected temperature region. This temperature region lies between 600° F. and 1100° F. with a preferred range from 800° F. to 1050° F. However, the preferred range may vary according to composition and fabrication techniques. Baths of molten lead or molten salt will serve well for this purpose. When the steel composition has been quenched to the proper temperature it is promptly worked to effect a substantial reduction of area before it has cooled below the selected temperature region into a region in which rapid transformation to bainite or other austenite decomposition products is possible. If the work is very severe, precautions should be taken that the metal is not heated by the energy of the working so as to approach or trespass in the temperature zone in which a transformation into pearlite is possible.

When the desired amount of deformation or work has been accomplished, the steel composition is quenched into the martensite transformation zone before any transformation of substance into austenite decomposition products takes place. This quench is into the martensite transformation zone and is sufficiently drastic to insure a predominantly martensitic microstructure. In most circumstances an ordinary water quench is adequate for this purpose.

The details of this heat treatment and working may more easily be visualized by reference to Figure 1 wherein the experience of the steel mass is traced by the heavy line originating in the upper left hand corner of the drawing and terminating on the abscissa near the ten minute graduation. The deformed horizontal portion of this curve indicates corresponding work.

The martensitic structure obtained by this quenching procedure must be tempered to obtain the optimum final results. Tempering may be accomplished at any temperature desired in the range of 150° F. to 750° F. depending upon the final properties desired. A progressive increase takes place in the ratio of yield strength to tensile strength as the tempering temperature increases. This ratio is about 0.71 at 150° and increases to 0.93 at 600° F. The preferred tempering range is 350° F. to 700° F.

A reference to the table supra will disclose a substantial silicon content in all of the alloys except the first three. The presence of this element is helpful in permitting tempering and use of the steel in the so-called blue-brittle range of about five hundred degrees to six hundred degrees Fahrenheit and to somewhat mitigate the deleterious effects of tempering upon the tensile strength. The carbon content of the alloys is important. Improvements

have been attained in steels ranging from 0.10 to 1.00 percent carbon. The preferred range is from 0.28 to 0.50 percent carbon.

It is preferred that the final product exhibit a very small grain size. The following table illustrates the effect of carbon content and deformation (percent reduction area) upon the grain size of a basic alloy containing two percent chromium, one and one-half percent silicon, one percent nickel, four tenths percent molybdenum and three-tenths percent vanadium.

| Deformation | Martensite Plate Size (Microns) |         |         |
|-------------|---------------------------------|---------|---------|
|             | 0.31% C                         | 0.41% C | 0.47% C |
| 15          | 3.2                             | 3.2     | 2.9     |
| 0.          | 2.7                             | 2.6     | 2.4     |
| 50.         | 2.0                             | 2.4     | 2.3     |
| 75.         | 1.9                             | 1.5     | 2.0     |
| 87.         | 1.5                             | 1.4     | 1.7     |
| 93.         |                                 |         |         |

In the practice of this invention it is preferred to rely upon chromium or nickel and chromium to stabilize the austenite against premature decomposition. However, it is to be understood that other elements known to have the same effect may also be so employed. Examples of such elements are boron, manganese and nitrogen.

To insure an adequate bay width between the pearlite transformation zone and the bainite transformation zone, additions of molybdenum may be made. A similar effect may also be had by additions of manganese, vanadium and tungsten.

We claim as our invention:

1. The process of forming and heat treating a steel product comprising heating a steel mass to a temperature sufficient to render the structure of the steel austenitic, the chemical composition of said steel mass being such that it exhibits a metastable austenite structure under conditions of substantial working when quenched from a temperature at which austenite is stable into a selected temperature region below the temperature at which austenite transforms into pearlite and above the temperature at which austenite transforms into bainite within the time necessary for the working process, quenching the austenitic mass sufficiently drastically to avoid any transformation into pearlite and to bring the mass to the selected temperature region without permitting any substantial transformation into bainite, performing a substantial amount of work upon the steel mass while maintaining the temperature of the mass within the selected region, said work being sufficient to effect a deformation of at least twenty-five percent at least locally, quenching the steel mass from the selected temperature region to a temperature at which the isothermal transformation products will be predominantly martensitic and tempering the martensitic structure so obtained to increase the yield point and to narrow the range between the yield point and the tensile strength whereby a fine grained martensitic product is obtained in which the martensitic grain size is substantially smaller than the martensitic grain size of the same steel if transformed directly to martensite without working of the metastable austenite.

2. The process of forming and heat treating a steel product comprising heating a steel mass to a temperature sufficient to render the structure of the steel austenitic, the chemical composition of said steel mass being such that it exhibits a metastable austenitic structure under conditions of substantial working when quenched from a temperature at which austenite is stable into a selected temperature region below the temperature at which austenite transforms into pearlite and above the temperature at which austenite transforms into bainite within the time necessary for the working process, quenching the austenitic mass sufficiently drastically to avoid any transformation into pearlite and to bring the mass to the selected temperature region without permitting any substantial

transformation into bainite, performing sufficient work upon the steel mass while maintaining the temperature of the steel mass within the selected region to deform the steel mass at least ninety percent, quenching the steel mass from the selected temperature region to a temperature at which the isothermal transformation products will be predominantly martensitic and tempering the martensitic structure so obtained to increase the yield point and to narrow the range between the yield point and the tensile strength whereby a fine grained martensitic product is obtained in which the martensitic grain size is substantially smaller than the martensitic grain size of the same steel if transformed directly to martensite without working of metastable austenite.

3. The process of forming and heat treating a steel product comprising heating a steel mass to a temperature sufficient to render the structure of the steel austenitic, the chemical composition of the steel including sufficient chromium that it exhibits a metastable austenitic structure under conditions of substantial working when quenched from a temperature at which austenite is stable into a selected temperature region below the temperature at which austenite transforms into pearlite and above the temperature at which austenite transforms into bainite within the time necessary for the working process, quenching the austenitic mass sufficiently drastically to avoid any transformation into pearlite and to bring the mass to the selected temperature region without permitting any substantial transformation into bainite, performing a substantial amount of work upon the steel mass while maintaining the temperature of the mass within the selected region, said work being sufficient to effect a deformation of at least twenty-five percent at least locally, quenching the steel mass from the selected temperature region to a temperature at which the isothermal transformation products will be predominantly martensitic and tempering the martensitic structure so obtained to increase the yield point and to narrow the range between the yield point and the tensile strength whereby a fine grained martensitic product is obtained in which the martensitic grain size is substantially smaller than the martensitic grain size of the same steel if transformed directly to martensite without working of the metastable austenite.

4. The process of forming and heat treating a steel product comprising heating a steel mass to a temperature sufficient to render the structure of the steel austenitic, the chemical composition of the steel including sufficient chromium that it exhibits a metastable austenitic structure under conditions of substantial working when quenched from a temperature at which austenite is stable into a selected temperature region below the temperature at which austenite transforms into pearlite and above the temperature at which austenite transforms into bainite within the time necessary for the working process, quenching the austenitic mass sufficiently to avoid any transformation into pearlite and to bring the mass to the selected temperature region without permitting any substantial transformation into bainite, performing sufficient work upon the steel mass while maintaining the temperature of the steel mass within the selected region to deform the steel mass at least ninety percent, quenching the steel mass from the selected temperature region to a temperature at which the isothermal transformation products will be predominantly martensitic and tempering the martensitic structure so obtained to increase the yield point and to narrow the range between the yield point and the tensile strength whereby a fine grained martensitic product is obtained in which the martensitic grain size is substantially smaller than the martensitic grain size of the same steel if transformed directly to martensite without working of metastable austenite.

5. The product of forming and heat treating a steel product comprising heating a steel mass to a temperature sufficient to render the structure of the steel austenitic,

the chemical composition of said steel mass being such that it exhibits a metastable austenitic structure under conditions of substantial working when quenched from a temperature at which austenite is stable into a selected temperature region below the temperature at which austenite transforms into pearlite and above the temperature at which austenite transforms into bainite within the time necessary for the working process, said selected temperature region extending from six hundred degrees Fahrenheit to one thousand one hundred degrees Fahrenheit, quenching the austenitic mass sufficiently drastically to avoid any transformation into pearlite and to bring the mass to the selected temperature region without permitting any substantial transformation into bainite, performing a substantial amount of work upon the steel mass while maintaining the temperature of the mass within the selected region, said work being sufficient to effect a deformation of at least twenty-five per cent at least locally, quenching the steel mass from the selected temperature region to a temperature at which the isothermal transformation products will be predominantly martensitic and tempering the martensitic structure so obtained to increase the yield point and to narrow the range between the yield point and the tensile strength whereby a fine grained martensitic product is obtained in which the martensitic grain size is substantially smaller than the martensitic grain size of the same steel if transformed directly to martensite without working of the metastable austenite.

6. The process of forming and heat treating a steel product comprising heating a steel mass to a temperature sufficient to render the structure of the steel austenitic, the chemical composition of said steel mass being such that it exhibits a metastable austenitic structure under conditions of substantial working when quenched from a temperature at which austenite is stable into a selected temperature region below the temperature at which austenite transforms into pearlite and above the temperature at which austenite transforms into bainite within the time necessary for the working process, said selected temperature region extending from six hundred degrees Fahrenheit to one thousand one hundred degrees Fahrenheit, quenching the austenitic mass sufficiently drastically to avoid any transformation into pearlite and to bring the mass to the selected temperature region without permitting any substantial transformation into bainite, performing sufficient work upon the steel mass while maintaining the temperature of the steel mass within the selected region to deform the steel mass at least ninety percent, quenching the steel mass from the selected temperature region to a temperature at which the isothermal transformation products will be predominantly martensitic and tempering the martensitic structure so obtained to increase the yield point and to narrow the range between the yield point and the tensile strength whereby a fine grained martensitic product is obtained in which the martensitic grain size is substantially smaller than the martensitic grain size of the same steel if transformed directly to martensite without working of metastable austenite.

7. The process of forming and heat treating a steel product comprising heating a steel mass to a temperature sufficient to render the structure of the steel austenitic, the chemical composition of the steel including sufficient chromium that it exhibits a metastable austenitic structure under conditions of substantial working when quenched from a temperature at which austenite is stable into a selected temperature region below the temperature at which austenite transforms into pearlite and above the temperature at which austenite transforms into bainite within the time necessary for the working process, said selected temperature region extending from six hundred degrees Fahrenheit to one thousand one hundred degrees Fahrenheit, quenching the austenitic mass sufficiently drastically to avoid any transformation into

pearlite and to bring the mass to the selected temperature region without permitting any substantial transformation into bainite, performing a substantial amount of work upon the steel mass while maintaining the temperature of the mass within the selected region, said work being sufficient to effect a deformation of at least twenty-five percent at least locally, quenching the steel mass from the selected temperature region to a temperature at which the isothermal transformation products will be predominantly martensitic and tempering the martensitic structure so obtained to increase the yield point and to narrow the range between the yield point and the tensile strength whereby a fine grained martensitic product is obtained in which the martensitic grain size is substantially smaller than the martensitic grain size of the same steel if transformed directly to martensite without working of the metastable austenite.

8. The process of forming and heat treating a steel product comprising heating a steel mass to a temperature sufficient to render the structure of the steel austenitic, the chemical composition of the steel including a sufficient chromium that it exhibits a metastable austenitic structure under conditions of substantial working when quenched from a temperature at which austenite is stable into a selected temperature region below the temperature at which austenite transforms into pearlite and above the temperature at which austenite transforms into bainite within the time necessary for the working process, said selected temperature region extending from six hundred degrees Fahrenheit to one thousand one hundred degrees Fahrenheit, quenching the austenitic mass sufficiently to avoid any transformation into pearlite and to bring the mass to the selected temperature region without permitting any substantial transformation into bainite, performing sufficient work upon the steel mass while maintaining the temperature of the steel mass within the selected region to deform the steel mass at least ninety percent, quenching the steel mass from the selected temperature region to a temperature at which the isothermal transformation products will be predominantly martensitic and tempering the martensitic structure so obtained to increase the yield point and to narrow the range between the yield point and the tensile strength whereby a fine grained martensitic product is obtained in which the martensitic grain size is substantially smaller than the martensitic grain size of the same steel if transformed directly to martensite without working of metastable austenite.

9. The process of forming and heat treating a steel product comprising heating a steel mass to a temperature sufficient to render the structure of the steel austenitic, the chemical composition of said steel mass being such that it exhibits a metastable austenitic structure under conditions of substantial working when quenched from a temperature at which austenite is stable into a selected temperature at which austenite transforms into pearlite and above the temperature at which austenite transforms into bainite within the time necessary for the working process, said selected temperature region extending from eight hundred degrees Fahrenheit to one thousand fifty degrees Fahrenheit, quenching the austenitic mass sufficiently drastically to avoid any transformation into pearlite and to bring the mass to the selected temperature region without permitting any substantial transformation into bainite, performing a substantial amount of work upon the steel mass while maintaining the temperature of the mass within the selected region, said work being sufficient to effect a deformation of at least twenty-five percent at least locally, quenching the steel mass from the selected temperature region to a temperature at which the isothermal transformation products will be predominantly martensitic and tempering the martensitic structure so obtained to increase the yield point and to narrow the range between the yield point and the tensile strength whereby a fine grained marten-

sitic product is obtained in which the martensitic grain size is substantially smaller than the martensitic grain size of the same steel if transformed directly to martensite without working of the metastable austenite.

5 10. The process of forming and heat treating a steel product comprising heating a steel mass to a temperature sufficient to render the structure of the steel austenitic, the chemical composition of said steel mass being such that it exhibits a metastable austenite structure under  
10 conditions of substantial working when quenched from a temperature at which austenite is stable into a selected temperature region below the temperature at which austenite transforms into pearlite and above the temperature at which austenite transforms into bainite within  
15 the time necessary for the working process, said selected temperature region extending from eight hundred degrees Fahrenheit to one thousand fifty degrees Fahrenheit, quenching the austenitic mass sufficiently drastically to avoid any transformation into pearlite and to bring the  
20 mass to the selected temperature region without permitting any substantial transformation into bainite, performing sufficient work upon the steel mass while maintaining the temperature of the steel mass within the selected region to deform the steel mass at least ninety percent, quenching  
25 the steel mass from the selected temperature region at which the isothermal transformation products will be predominantly martensitic and tempering the martensitic structure so obtained to increase the yield point and to narrow the range between the yield point and the tensile  
30 strength whereby a fine grained martensitic product is obtained in which the martensitic grain size is substantially smaller than the martensitic grain size of the same steel if transformed directly to martensite without working of metastable austenite.

35 11. The process of forming and heat treating a steel  
product comprising heating a steel mass to a tempera-  
ture sufficient to render the structure of the steel austen-  
itic, the chemical composition of the steel including  
sufficient chromium that it exhibits a metastable austen-  
itic structure under conditions of substantial working  
40 when quenched from a temperature at which austenite  
is stable into a selected temperature region below the  
temperature at which austenite transforms into pearlite  
and above the temperature at which austenite transforms  
45 into bainite within the time necessary for the working  
process, said selected temperature region extending from  
eight hundred degrees Fahrenheit to one thousand fifty  
degrees Fahrenheit, quenching the austenitic mass suffi-  
ciently drastically to avoid any transformation into pearl-  
ite 50 and to bring the mass to the selected temperature  
region without permitting any substantial transformation  
into bainite, performing a substantial amount of work  
upon the steel mass while maintaining the temperature  
of the mass within the selected region, said work being  
55 sufficient to effect a deformation of at least twenty-five  
percent at least locally, quenching the steel mass from  
the selected temperature region to a temperature at which  
the isothermal transformation products will be predomi-  
nantly martensitic and tempering the martensitic struc-  
ture 60 so obtained to increase the yield point and to narrow  
the range between the yield point and the tensile strength  
whereby a fine grained martensitic product is obtained in  
which the martensitic grain size is substantially smaller  
than the martensitic grain size of the same steel if trans-  
formed directly to martensite without working of the  
65 metastable austenite.

12. The process of forming and heat treating a steel product comprising heating a steel mass to a temperature sufficient to render the structure of the steel austenitic, the chemical composition of the steel including sufficient chromium that it exhibits a metastable austenitic structure under conditions of substantial working when quenched from a temperature at which austenite is stable into a selected temperature region below the temperature at which austenite transforms into pearlite and

above the temperature at which austenite transforms into bainite within the time necessary for the working process, said selected temperature region extending from eight hundred degrees Fahrenheit to one thousand fifty degrees Fahrenheit, quenching the austenitic mass sufficiently to avoid any transformation into pearlite and to bring the mass to the selected temperature region without permitting any substantial transformation into bainite, performing sufficient work upon the steel mass while maintaining the temperature of the steel mass within the selected region to deform the steel mass at least ninety percent, quenching the steel mass from the selected temperature region to a temperature at which the isothermal transformation products will be predominantly martensitic and tempering the martensitic structure so obtained to increase the yield point and to narrow the range between the yield point and the tensile strength, whereby a fine grained martensitic product is obtained in which the martensitic grain size is substantially smaller than the martensitic grain size of the same steel if transformed directly to martensite without working of metastable austenite.

13. The process of forming and heat treating a steel product comprising heating a steel mass to a temperature sufficient to render the structure of the steel austenitic, the chemical composition of the said steel mass being such that it exhibits a metastable austenitic structure under conditions of substantial working when quenched from a temperature at which austenite is stable into a selected temperature region below the temperature at which austenite transforms into pearlite and above the temperature at which austenite transforms into bainite within the time necessary for the working process, said temperature region extending from six hundred degrees Fahrenheit to one thousand one hundred degrees Fahrenheit, quenching the austenitic mass sufficiently drastically to avoid any transformation into pearlite and to bring the mass to the selected temperature region without permitting any substantial transformation into bainite, performing a substantial amount of work upon the steel mass while maintaining the temperature of the mass within the selected temperature region, said work being sufficient to effect a deformation of at least twenty-five percent at least locally, quenching the steel mass from the selected temperature region to a temperature at which the isothermal transformation products will be predominantly martensitic and tempering the martensitic structure so obtained at a temperature falling within the range of one hundred fifty degrees Fahrenheit to seven hundred fifty degrees Fahrenheit to increase the yield point and to narrow the range between the yield point and the tensile strength, whereby a fine grained martensitic product is obtained in which the martensitic grain size is substantially smaller than the martensitic grain size of the same steel if transformed directly to martensite without working of the metastable austenite.

14. The process of forming and heat treating a steel product comprising heating a steel mass to a temperature sufficient to render the structure of the steel austenitic, the chemical composition of the said steel mass being such that it exhibits a metastable austenitic structure under conditions of substantial working when quenched from a temperature at which austenite is stable into a selected temperature region below the temperature at which austenite transforms into pearlite and above the temperature at which austenite transforms into bainite within the time necessary for the working process, said temperature region extending from eight hundred degrees Fahrenheit to one thousand fifty degrees Fahrenheit, quenching the austenitic mass sufficiently drastically to avoid any transformation into pearlite and to bring the mass to the selected temperature region without permitting any substantial transformation into bainite, performing a substantial amount of work upon the steel mass while maintaining the temperature of the mass with-

in the selected temperature region, said work being sufficient to deform the steel mass at least ninety percent, quenching the steel mass from the selected temperature region to a temperature at which the isothermal transformation products will be predominantly martensitic and tempering the martensitic structure so obtained at a temperature falling within the range of three hundred fifty to seven hundred degrees Fahrenheit to increase the yield point and to narrow the range between the yield point and the tensile strength, whereby a fine grained martensitic product is obtained in which the martensitic grain size is substantially smaller than the martensitic grain size of the same steel if transformed directly to martensite without working of the metastable austenite.

15. 15. The process of forming and heat treating a steel product comprising heating a steel mass to a temperature sufficient to render the structure of the steel austenitic, the chemical composition of the said steel mass including sufficient chromium so that it exhibits a metastable austenitic structure under conditions of substantial working when quenched from a temperature at which austenite is stable into a selected temperature region below the temperature at which austenite transforms into pearlite and above the temperature at which austenite transforms into bainite within the time necessary for the working process, said temperature region extending from six hundred degrees Fahrenheit to one thousand one hundred degrees Fahrenheit, quenching the austenitic mass sufficiently drastically to avoid any transformation into pearlite and to bring the mass to the selected temperature region without permitting any substantial transformation into bainite, performing a substantial amount of work upon the steel mass while maintaining the temperature of the mass within the selected temperature region, said work being sufficient to effect a deformation of at least twenty-five percent at least locally, quenching the steel mass from the selected temperature region to a temperature at which the isothermal transformation products will be predominantly martensitic and tempering the martensitic structure so obtained at a temperature falling within the range of one hundred fifty to seven hundred fifty degrees Fahrenheit to increase the yield point and to narrow the range between the yield point and the tensile strength, whereby a fine grained martensitic product is obtained in which the martensitic grain size is substantially smaller than the martensitic grain size of the same steel if transformed directly to martensite without working of the metastable austenite.

16. The process of forming and heat treating a steel product comprising heating a steel mass to a temperature sufficient to render the structure of the steel austenitic, the chemical composition of the said steel mass including sufficient chromium so that it exhibits a metastable austenitic structure under conditions of substantial working when quenched from a temperature at which austenite is stable into a selected temperature region below the temperature at which austenite transforms into pearlite and above the temperature at which austenite transforms into bainite within the time necessary for the working process, said temperature region extending from six hundred degrees Fahrenheit to one thousand one hundred degrees Fahrenheit, quenching the austenitic mass sufficiently drastically to avoid any transformation into pearlite and to bring the mass to the selected temperature region without permitting any substantial transformation into bainite, performing a substantial amount of work upon the steel mass while maintaining the temperature of the mass within the selected temperature region, said work being sufficient to deform the steel mass at least ninety percent, quenching the steel mass from the selected temperature region to a temperature at which the isothermal transformation products will be predominantly martensitic and tempering the martensitic structure so obtained at a temperature falling within the range of one hundred fifty to

seven hundred fifty degrees Fahrenheit to increase the yield point and to narrow the range between the yield point and the tensile strength, whereby a fine grained martensitic product is obtained in which the martensitic grain size is substantially smaller than the martensitic grain size of the same steel if transformed directly to martensite without working of the metastable austenite.

17. The process of producing a steel product having a minimum dimension of at least one-eighth inch, the microstructure of which is tempered martensite, comprising selecting a steel composition exhibiting a metastable austenitic structure under conditions of working when quenched from a temperature at which austenite is stable into a selected temperature region below the temperature at which austenite transforms into pearlite and above the temperature at which austenite transforms into bainite within the time necessary for the working process, heating the steel composition to render it stably austenitic, quenching the austenitized hardenable alloy steel composition sufficiently drastically to avoid any transformation into pearlite and to bring the composition to the selected temperature region, performing a substantial amount of work upon the steel composition while maintaining it in said selected temperature region until the substantial amount of work has been completed, said work being sufficient to effect a deformation of at least twenty-five percent, quenching the composition from the selected temperature region to a temperature at which the transformation products will consist essentially of martensite, said quenching operation being sufficiently drastic to insure a structure consisting essentially of martensite, and tempering the martensitic structure so obtained to narrow the range between the yield point and the tensile strength and to enhance the ductility, whereby a product is obtained in which the martensitic grain size is not over one-half of the martensitic grain size of the same steel if transformed directly to martensite without working of the metastable austenite.

18. The process of producing a steel product having a minimum dimension of at least one-eighth inch, the microstructure of which is tempered martensite, comprising selecting a steel composition comprising carbon 0.10 percent to 0.80 percent, nickel 2 percent to 6 percent, and chromium 0.75 percent to 3.0 percent and exhibiting a metastable austenitic structure under conditions of working when quenched from a temperature at which austenite is stable into a selected temperature region below the temperature at which austenite transforms into pearlite and above the temperature at which austenite transforms into bainite within the time necessary for the working process, heating the steel composition to render it stably austenitic, quenching the austenitized hardenable alloy steel composition sufficiently drastically to avoid any transformation into pearlite and to bring the composition to the selected temperature region, performing a substantial amount of work upon the steel composition while maintaining it in said selected temperature region until the substantial amount of work has been completed, said work being sufficient to effect a deformation of at least twenty-five percent, quenching the composition from the selected temperature region to a temperature at which the transformation products will consist essentially of martensite, said quenching operation being sufficiently drastic to insure a structure consisting essentially of martensite, and tempering the martensitic structure so obtained.

19. The process of producing a steel product having a minimum dimension of at least one-eighth inch, the microstructure of which is tempered martensite, comprising selecting a steel composition exhibiting a metastable austenitic structure under conditions of working when quenched from a temperature at which austenite is stable into a selected temperature region below the temperature at which austenite transforms into pearlite and above the temperature at which austenite transforms into bainite within the time necessary for the working process, said selected temperature region comprising the range extending from six hundred degrees Fahrenheit to one thousand one hundred degrees Fahrenheit, heating the steel composition to render it stably austenitic, quenching the austenitized composition sufficiently drastically to avoid any transformation into pearlite and to bring the composition to the selected temperature region, performing a substantial amount of work upon the steel composition while maintaining it in said selected temperature region until the substantial amount of work has been completed, said work being sufficient to effect a deformation of at least twenty-five percent at least locally, quenching the composition from the selected temperature region to a temperature at which the transformation products will consist essentially of martensite, said quenching operation being sufficiently drastic to insure a structure consisting essentially of martensite, and tempering the martensitic structure so obtained at a temperature in the range of one hundred fifty degrees Fahrenheit to seven hundred fifty degrees Fahrenheit.

20. The product produced by the process of claim 19, which product is metallographically indistinguishable from that depicted in Figure 1 and which consists essentially of a very fine grained tempered martensite.

21. The product produced by the process of claim 1, which product consists essentially of a very fine grained tempered martensite.

22. The process of producing a steel product having a minimum dimension of at least one-eighth inch, the microstructure of which is tempered martensite, comprising selecting a steel composition exhibiting a metastable austenitic structure under conditions of working when quenched from a temperature at which austenite is stable into a selected temperature region below the temperature at which austenite transforms into pearlite and above the temperature at which austenite transforms into bainite within the time necessary for the working process, heating the steel composition to render it stably austenitic, quenching the austenitized hardenable alloy steel composition sufficiently drastically to avoid any transformation into pearlite and to bring the composition to the selected temperature region, performing a substantial amount of work upon the steel composition while maintaining it in said selected temperature region until the substantial amount of work has been completed, said work being sufficient to effect a deformation of at least ninety percent, quenching the composition from the selected temperature region to a temperature at which the transformation products will consist essentially of martensite, said quenching operation being sufficiently drastic to insure a structure consisting essentially of martensite, and tempering the martensitic structure so obtained.

UNITED STATES PATENT OFFICE  
CERTIFICATE OF CORRECTION

April 26, 1960

Patent No. 2,934,463

Duane J. Schmatz et al.

It is hereby certified that error appears in the printed specification of the above numbered patent requiring correction and that the said Letters Patent should read as corrected below.

Column 2, line 57, after "tempering" insert -- tempera-  
ture --; column 7, line 44, for "in" read -- is --.

Signed and sealed this 20th day of December 1960.

(SEAL)

Attest:

KARL H. AXLINE  
Attesting Officer

ROBERT C. WATSON  
Commissioner of Patents